

## UNITED STATES PATENT OFFICE

2,207,916

PRODUCTION OF PHOTOGRAPHIC COLOR  
SOUND FILMS

John Eggert, Leipzig, Gerd Heymer, Wolfen, Kreis Bitterfeld, and Werner Schultze, Dessau in Anhalt, Germany, assignors, by mesne assignments, to General Aniline & Film Corporation, New York, N. Y., a corporation of Delaware

No Drawing. Application June 19, 1937, Serial No. 149,206. In Germany August 14, 1936

## 1 Claim. (Cl. 95-2)

Our present invention relates to photographic sound films and more particularly to photographic color sound films.

One of its objects is to provide a process of producing color sound films. Further objects will be seen from the detailed specification following hereafter.

It is known that in certain process for producing color sound films the sound track must receive special consideration. If the sound track has been produced in color on a colorless or colored ground the track itself must be opaque to that light for which the scanning photo-cell is sensitive and further all the remaining color layers which if desired cover the region of the sound strip in even coloration, must be fully transparent for this region. This is the case, for example, in so-called silver bleaching-out processes, in which the photographic layers contain dyestuffs and metallic silver or compounds of these and in which by treatment with certain baths, particularly where the silver or certain compounds of the silver are to be found, the color is destroyed. The reproduction of the sound by means of a pure color image without silver introduces certain difficulties, since the dyestuff has frequently too little opacity and diminution of tone as a result. It has been proposed, therefore, as in the case of other color film processes, to produce the sound track itself as a silver image in the colored layers. In order to make this silver color bleaching-out process possible the film must be dried after the developing and fixing of the sound strip and then the sound track must be protected by a varnish impermeable to water before the treatment in the subsequent baths for bleaching the color. This process is inconvenient and very difficult to practice in the case of continuous production. Moreover, the requisite varnishing may be a source of disturbance owing to perforations in the varnished layer, whereby the bleaching-out process is not complete and in consequence the sound track develops a discordant murmur; moreover, if the varnish dries in a wavy form or later becomes cracked like, disturbances are introduced.

This invention relates to a process whereby the manufacture is simplified and the possible sound disturbances are diminished as much as may be, and comprises the conversion, after the production of the silver images, of the silver of the sound strip into a compound, which on the one hand must obviously be opaque in the region of the spectrum to which the scanning device is sensitive and on the other hand must have the

characteristic that in the following bleaching baths there is no further action on this color, so that the application of the varnish, with its injurious consequences, is unnecessary.

For example, the following procedure may be cited as useful: after developing, fixing and washing the picture strip and the sound strip the sound track and this only is treated in the following solution:

## 10 Portion 1

|                                                      |       |      |
|------------------------------------------------------|-------|------|
| Potassium ferricyanide                               | grams | 10   |
| Potassium bichromate solution of 1 per cent strength | cc    | 1.3  |
| Water                                                | litre | 1 15 |

## 20 Portion 2

|                   |       |    |
|-------------------|-------|----|
| Iron ammonia alum | grams | 21 |
| Water             | litre | 1  |

## 20 Portion 3

|             |       |    |
|-------------|-------|----|
| Oxalic acid | grams | 25 |
| Water       | litre | 1  |

The solution for the treatment is made by mixing equal volumes of Portions 1, 2 and 3. The limitation of the action of this bath to the sound strip is secured in the known manner, that is to say the film dips in the solution only in so far as the sound strip is covered or the solution is applied to the sound strip by means of rollers, bands of a spongy structure, spraying nozzles or the like, care being taken that by inclination of the edge of the film in question the solution is prevented from running over the picture strip. The Prussian Blue image thus produced is sufficiently opaque to the infra-red for which the photo-cells preferably used at the present time are chiefly sensitive and this coloring matter does not change in the subsequent bleaching baths.

Another example is as follows: After developing, fixing and washing of the picture strip and sound strip the latter is treated as described above in the following solution:

|                                                         |    |
|---------------------------------------------------------|----|
| Lead nitrate solution of 10 per cent strength           | 15 |
| Potassium ferricyanide solution of 10 per cent strength | 10 |
| Nitric acid of 10 per cent strength                     | 1  |
| Water                                                   | 75 |

After a treatment for about 5 minutes the film without being washed is transferred to a bath of nitric acid of 10 per cent strength and then washed for about two minutes and treated with

the following bath to produce an indifferent toning:

|                                                      |    |     |
|------------------------------------------------------|----|-----|
| Cobalt nitrate solution of 10 per cent strength      | 30 | cc. |
| 5 Potassium bromide solution of 10 per cent strength | 20 |     |
| Nitric acid of 10 per cent strength                  | 1  |     |
| Water                                                | 70 |     |

10 This toning may be applied if desired after the first development and before the first fixing if care is taken to interrupt the development by means of a suitable bath.

15 Since a portion of the light for which the photo-cell is sensitive is absorbed in the film containing coloring matters, particularly in the blue-green portion, it is frequently advantageous to destroy this coloring matter and particularly the blue-green color in order that the reproduction of the sound may be possible with a more feeble source of light.

20 For this purpose the sound track may be produced in known manner on that side of the film which does not contain the blue-green portion and the side containing the blue-green portion is diffusely illuminated opposite the sound track so that in the bleaching bath the blue-green coloring matter is destroyed. Instead of treating the sound strip in a bath, however, it is possible to destroy the coloring matter, particularly the blue-green portion without attacking the substance of the sound track. In this

case the sound track may be either on the same side as the blue-green portion or on the opposite side.

25 For example, if the film carries as the blue-green dyestuff Brilliant Benzo Fast Green after the conversion of the silver of the sound track into Prussian Blue the sound strip may be treated with a solution containing per liter of water 8 grams of potassium bichromate and 16 cc. of concentrated sulfuric acid. While the Prussian Blue is not attacked by this solution the dye-stuff in the blue-green layer is very rapidly destroyed. Just as in the above described conversion of the silver of the sound track into another substance care must obviously be taken that the bath can affect only the sound track and not the pictures.

10 What we claim is:

15 A process of producing subtractive color pictures with a sound track which comprises copying the picture and the sound onto a subtractive silver color bleaching-out film, developing, fixing, washing the picture strip and the sound strip, transforming the silver image of the sound track to a ferric ferrocyanide image, bleaching 20 out the dyestuff by means of a bath usual in silver color bleaching-out processes, and removing the superfluous silver.

JOHN EGGERT. 30  
GERD HEYMER.  
WERNER SCHULTZE.